

1

 3,159,678  
**NITRAMINES**

Milton B. Frankel, Pasadena, and Karl Klager, Monrovia, Calif., assignors to Aerojet-General Corporation, Azusa, Calif., a corporation of Ohio  
 No Drawing. Filed June 13, 1957, Ser. No. 666,276  
 9 Claims. (Cl. 260—583)

This invention relates to new compositions of matter and to their preparation. More particularly, the invention relates to nitramines of the following general formula:



wherein R is a hydrogen, alkyl, or nitroalkyl radical; A is an alkylene radical; and R' is a hydrogen, nitro, alkyl, or nitroalkyl radical.

The nitramines of this invention react with nitric acid according to the method disclosed in our copending U.S. patent application Serial No. 666,274, now U.S. Patent 3,098,873, filed concurrently with the present application, to form high energy nitramines such as, 3,6-diaza-1,1,1,3,6-pantanitroheptane, which are useful as high explosives and can be used in any conventional explosive missile, projectile, rocket, or the like, as the main explosive charge. An example of such a missile is disclosed in United States Patent 2,470,162, issued May 17, 1949. One way of using the high explosives which can be prepared from the nitramines of the present invention in a device such as that disclosed in United States Patent No. 2,470,162, is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact- or time fuse-mechanism firing a detonating explosive such as lead azide or mercury fulminate.

The novel nitramine compounds of this invention are prepared by condensing nitraza amines with  $\beta$ -geminal polynitro alcohols in accordance with the general reaction scheme set forth below:



wherein R, A, and R' are as previously defined.

To more clearly illustrate our invention, the following example is presented. It should be understood that this example is presented merely as a means of illustration and is not intended to limit the scope of the invention in any way.

**Example I.—Preparation of 3,6-Diaza-1,1,1,6-Tetranitroheptane**

To a mixture of 25.5 g. (0.16 mole) of 3-nitraza-1-butyl ammonium chloride, 29.7 g. (0.16 mole) of 2,2,2-trinitroethanol and 150 ml. of distilled water, was added 50 ml. of water containing 6.7 g. (0.16 mole) of sodium hydroxide in solution. An orange-colored oil formed which was extracted with tetrahydrofuran and subsequently dried and concentrated in vacuo to yield, as the final product, 29 g. (64.3%) of a red oil.

2

Optimum results are obtained from the condensation reaction of this invention when it is carried out at a pH below about 8 and preferably within the range from about 4 to about 8.

5 Reaction temperature is non-critical in the condensation reaction of this invention, the only effect of temperature variation being a corresponding increase or decrease in reaction rate.

As a matter of convenience, the free nitraza amine starting materials of this invention are preferably generated in situ from their corresponding strong mineral acid salts by neutralizing said strong mineral acid salts with inorganic basic salts, as for example hydroxides or carbonates, or weak organic acid salts, as for example acetates, of alkali or alkaline earth metals as more fully disclosed in assignee's copending U.S. patent application Serial No. 666,273, now U.S. Patent 3,000,954, filed concurrently with the present application. For reasons of convenience and economy we prefer to use sodium hydroxide as our free nitraza amine generating agent but other suitable agents such as, for example, calcium hydroxide, magnesium hydroxide, sodium carbonate, sodium acetate, etc., can be used for this purpose if desired.

Any of the strong mineral acid salts such as nitric acid, hydrochloric acid, etc., salts of our amine starting materials can be used in the practice of our invention as taught herein.

Nitraza amine salts useful in the practice of this invention are prepared by reacting a corresponding nitraza isocyanate such as, for example, 3-nitraza-1-butyl isocyanate, with an aqueous solution of a strong mineral acid, as more fully disclosed in assignee's copending U.S. patent application Serial No. 666,273, now U.S. Patent 3,000,954, filed concurrently with the present application.

35 The  $\beta$ -geminal polynitro alcohol reaction of this invention can be 2,2-dinitro-1-ethanol; 2,2,2-trinitroethanol; a compound in which R' is an alkyl radical as, for example, 2,2-dinitro-1-butanol; or a compound in which R' is a nitroalkyl radical as, for example, the 2,2,4,4-tetranitro-1-butanol disclosed in assignee's copending U.S. patent application Serial No. 371,149, filed July 29, 1953, now abandoned. These  $\beta$ -geminal polynitro alcohols are prepared by condensing labile hydrogen containing nitroalkanes, such as, trinitromethane, with formaldehyde.

40 45 It will be appreciated that a wide variety of compounds can be prepared in accordance with the method of our invention. For example, the strong mineral acid salts of 4-nitraza-1-hexylamine; 3-aza-3,5,5-trinitro-1-hexylamine; and 3-nitraza-1-butylamine react with 2,2-dinitro-1-ethanol; 2,2-dinitro-1-propanol; and 2,2,4,4-tetranitro-1-butanol, respectively, to produce 3,7-diaza-1,1,7-trinitrononane; 4,7-diaza-2,2,7,9,9-pantanitrodecane; and 5,8-diaza-1,1,3,3,8-pantanitrononane, respectively. Other members of this new series of compounds are prepared 50 55 simply by reacting appropriate starting materials.

We claim:

1. As a composition of matter, a nitramine having the general formula:



60 65 wherein R is an alkyl radical and A is an alkylene radical.

2. As a composition of matter, 3,6-diaza-1,1,1,6-tetranitroheptane having the structural formula:



3. The method of preparing a nitramine having the general formula:



5

which comprises condensing a nitraza amine having the general formula:



10

with a  $\beta$ -geminal polynitro alcohol having the general formula:



15

wherein R is a radical selected from the group consisting of hydrogen, alkyl, and nitroalkyl radicals; A is an alkylene radical; and R' is a radical selected from the group consisting of hydrogen, nitro, alkyl, and nitroalkyl radicals.

4. The method of claim 3 in which the nitraza amine is generated in situ.

5. The method of claim 3 in which the nitraza amine is generated in situ from a strong mineral acid salt thereof by neutralizing said salt with an aqueous solution of a salt selected from the group consisting of the inorganic basic salts and the weak organic acid salts of the alkali and alkaline earth metals.

6. The method of preparing a nitramine having the general formula:



which comprises condensing a nitraza amine having the general formula:



with 2,2,2-trinitroethanol; wherein R is an alkyl radical and A is an alkylene radical.

7. The method of claim 6 in which the nitraza amine is generated in situ.

8. The method of preparing 3,6-diaza-1,1,1,6-tetranitroheptane which comprises condensing 3-nitraza-1-butyl amine with 2,2,2-trinitroethanol.

9. The method of claim 8 in which the 3-nitraza-1-butyl amine is generated in situ.

#### References Cited in the file of this patent

#### UNITED STATES PATENTS

2,731,460 Schenck et al. ----- Jan. 17, 1956

#### OTHER REFERENCES

Textbook of Organic Chemistry, Wertheim, 2nd Ed., The Blakiston Co., Philadelphia, page 308.

20

30